

# UNITED STATES PATENT OFFICE.

FELIX A. ELLIOTT, OF ROCHESTER, NEW YORK, ASSIGNOR TO EASTMAN KODAK COMPANY, OF ROCHESTER, NEW YORK, A CORPORATION OF NEW YORK.

## PHOTOGRAPHIC BATH.

1,411,687.

Specification of Letters Patent.

REISSUED  
Patented Apr. 4, 1922.

No Drawing.

Application filed April 13, 1921. Serial No. 460,995.

To all whom it may concern:

Be it known that I, FELIX A. ELLIOTT, a citizen of the United States of America, residing at Rochester, in the county of Monroe and State of New York, have invented certain new and useful Improvements in Photographic Baths, of which the following is a full, clear, and exact specification.

This invention relates to photographic 10 baths and more particularly to acid fixing baths.

It is well known that solutions of sodium thiosulfate, used for the removal from photographic emulsions of undeveloped silver salts, 15 should be acidified. Alum is generally added to the fixing bath for the purpose of hardening the gelatine, and if the bath is or becomes alkaline, or too weakly acid, there is a tendency for aluminium compounds to precipitate alumina or aluminium salts. On the 20 other hand, if the bath is too acid, sulfur is precipitated from the sodium thiosulfate. It is necessary, however, to have enough acid present to neutralize the considerable 25 amounts of alkali brought over from the developer.

In an attempt to satisfy these requirements, organic acids are generally used because they are but slightly dissociated in 30 solution and hence render the bath sufficiently acid, while since the total amount of alkali which can be neutralized depends on the total amount of acid present, the undissociated acid acts as a reserve from which 35 the acidity, that is the hydrogen ion concentration, of the bath is replenished or maintained with gradually decreasing strength until the acidity of the bath becomes less than is desirable.

40 The amounts of these organic acids that can be added, however, are not sufficient to maintain the acidity of the bath within the desired limits during the life of the bath and it is necessary either to add acid or discard the bath.

I have discovered that the acidity of such a bath may be maintained within the desired limits for the full life of the bath by the "buffer action" of certain substances in 50 solution. By the full life of the bath I mean until the sodium thiosulfate is exhausted. By "buffer action" is meant the ability of a solution to resist change in its hydrogen ion concentration through the addition or loss

of acid or alkali. The unit by which hydrogen ion concentration is measured is defined as represented by the symbol pH or  $P_H$ . I have here adopted the former symbol consistently with its use in the Journal of Biological Chemistry. Full explanation of the theory underlying the "buffer action" referred to above is contained in the literature, and it is unnecessary here to review it. Reference is made particularly to the comparatively simple explanation found in "The Determination of Hydrogen Ions" by Clark, published 1920, by the Williams and Wilkins Company, Baltimore, Maryland, and to the extensive bibliography contained therein.

For a neutral solution, the expression  $pH=7$  is approximately correct, and it has been found that the fixing bath should have an acidity or hydrogen ion concentration not greater than  $pH=4$  and not less than 75  $pH=6.5$  or, preferably,  $pH=6$ . It is possible by applying known ionization formulæ to compute the required amount of suitable buffers, that is substances capable by dissociation in accordance with the law of mass action of maintaining the acidity of the fixing bath within the desired limits. The weaker acids, that is, ones which are but partially dissociated in solution, such as the organic acids, for instance acetic acid, citric acid, formic acid and others, have been found to be admirably adapted for use in such a bath. As the buffer material, I have found particularly useful the neutral salts of the alkali metals (including ammonium) of the acid used. Thus acetic acid and sodium acetate, or citric acid and sodium citrate may be used together with satisfactory results. The buffer material should be slightly acid rather than slightly neutral. 95 Thus sodium dihydrogen phosphate is a suitable buffer, being slightly acid, while disodium hydrogen phosphate is unsuitable. Boric acid can also be used as a buffer for a stronger acid such as acetic acid.

100 The following formula is a typical one embodying my invention:

|                       |      |       |     |
|-----------------------|------|-------|-----|
| Sodium thiosulfate    | 300  | grams |     |
| Sodium sulfite        | 50   | grams | 105 |
| Acetic acid (glacial) | 2.4  | grams |     |
| Sodium acetate        | 10.5 | grams |     |
| Water to              | 1    | liter |     |

If desired there may be added a suitable hardener such as potash alum, 60 grams.

Another formula is:

|   |                    |           |
|---|--------------------|-----------|
| 5 | Sodium thiosulfate | 100 grams |
|   | Sodium sulfite     | 20 grams  |
|   | Citric acid        | 4 grams   |
|   | Sodium citrate     | 6 grams   |
|   | Water              | 600 cc.   |

10 to which may be added a suitable hardener.

While I have endeavored to point out the principles of my invention and to give preferred examples thereof, it is to be understood that there is possible a wide range of

15 equivalents, the use of which I contemplate as within the scope of my invention as defined in the appended claims.

When in the claims I refer to the hydrogen ion concentration being maintained at a pre-

20 determined strength, I do not mean that it is maintained precisely constant during the entire life of the bath, but that it is maintained within certain reasonably narrow limits, at a value such that the bath is useful.

25 Having thus described my invention, what I claim as new and desire to secure by Letters Patent is:

1. A photographic bath comprising in solution a substance capable of affecting a photographically sensitive salt, an acid and a substance capable of maintaining the hydrogen ion concentration of the bath at a predetermined strength by dissociation.

30 2. A photographic bath comprising in solution a substance capable of affecting a photographically sensitive salt, an acid that is but slightly dissociated in solution and a substance capable of maintaining the hydrogen ion concentration of the bath at a predetermined strength by dissociation.

35 3. A photographic bath comprising in solution a solvent for silver halides, an acid and a substance capable of maintaining the hydrogen ion concentration of the bath at a predetermined strength by dissociation.

40 4. A photographic bath comprising in solution a solvent for silver halides, an acid that is but slightly dissociated in solution, and a substance capable of maintaining the hydrogen ion concentration of the bath at a predetermined strength by dissociation.

45 5. A photographic fixing bath comprising an acid solution of sodium thiosulfate and a substance capable of maintaining the hydrogen ion concentration of the bath at a predetermined strength by dissociation.

50 6. A photographic fixing bath comprising an acid aqueous solution of sodium thiosulfate and a substance capable of maintaining by dissociation the hydrogen ion concentration of the bath between pH=4 and pH=6.5.

55 7. A photographic fixing bath comprising

an acid aqueous solution of sodium thiosulfate and an acetate.

8. A photographic fixing bath comprising an acid aqueous solution of sodium thiosulfate and an acetate, the acetate being capable of maintaining the hydrogen ion concentration of the bath between pH=4 and pH=6.5.

9. A photographic fixing bath comprising in aqueous solution sodium thiosulfate, an acid and a neutral salt capable of maintaining the hydrogen ion concentration of the bath at a predetermined strength by dissociation.

10. A photographic fixing bath comprising in solution sodium thiosulfate, an organic acid and a salt of said acid capable of maintaining the hydrogen ion concentration 80 of the bath at a predetermined strength by dissociation.

11. A photographic fixing bath comprising in aqueous solution sodium thiosulfate, an organic acid, and a neutral salt of said 85 acid capable of maintaining the hydrogen ion concentration of the bath at a predetermined strength by dissociation.

12. A photographic fixing bath comprising in aqueous solution sodium thiosulfate, 90 an acid that is but slightly dissociated in solution, and a substance capable of maintaining the hydrogen ion concentration of the bath at a predetermined strength by dissociation.

95 13. A photographic fixing bath comprising in aqueous solution sodium thiosulfate, acetic acid and a substance capable of maintaining the hydrogen ion concentration of the bath at a predetermined strength by dissociation.

14. A photographic fixing bath comprising an acid aqueous solution of sodium thiosulfate and sodium acetate.

15. A photographic fixing bath comprising in aqueous solution sodium thiosulfate, 105 acetic acid and an acetate.

16. A photographic fixing bath comprising in aqueous solution sodium thiosulfate, acetic acid and sodium acetate, there being 110 present a sufficient quantity of sodium acetate to maintain by dissociation the hydrogen ion concentration of the bath between pH=4 and pH=6.5.

115 17. A photographic bath with a predetermined hydrogen ion concentration, and containing a substance capable of affecting photographically sensitive salts and a substance capable of maintaining the hydrogen ion concentration within predetermined limits 120 during the life of the bath.

Signed at Rochester, New York, this 7th day of April, 1921.

FELIX A. ELLIOTT.